

106/81  
Patented July 9, 1929.

1,720,356

# UNITED STATES PATENT OFFICE.

ALFRED R. WILLARD, OF EAST CLEVELAND, OHIO, ASSIGNOR TO WILLARD STORAGE BATTERY COMPANY, OF CLEVELAND, OHIO, A CORPORATION OF WEST VIRGINIA.

## COATING MATERIAL FOR METAL MOLDS.

No Drawing.

Application filed September 27, 1926. Serial No. 138,186.

This invention relates to a compound for coating metal molds, my invention having special utility when applied to molds used in making lead or lead antimony storage battery grids.

Considerable difficulty is encountered in casting storage battery grids because of the filmy, intricate nature of the grids and the fact that the grids are formed of material which melts at a low temperature and, therefore, tends to congeal quickly. In order that a cast grid may be perfect, it is, of course, essential that it be completely filled out, but since a grid is composed of a great number of ribs having considerable length and exceedingly small in cross section, to obtain a perfect grid the molten lead must flow through all the minor interstices or small rib forming passageways and must reach the parts of the mold cavity most remote from the pouring point before the metal congeals or has any considerable tendency to congeal.

Accordingly, it has been customary to apply to the faces of both parts of the mold a coating which has the double function of insulating the molten metal from the metal mold and preventing the grid from sticking to the mold. Powdered soapstone is commonly employed for this purpose, and in some instances lamp black has been employed but neither of the above substances has been entirely satisfactory, and in fact each has distinct disadvantages. For example, when either soapstone or lamp black is employed, the room or building in which the casting is done becomes permeated with the soapstone powder or with soot, since both substances are finely divided and are carried to the remotest parts of the building. Furthermore, considerable skill is required in the application of these substances, particularly soapstone dust, for if too much is applied or if it is not applied evenly the grid is likely to be ruined as the molten metal flowing through the mold cavity gathers up the dust or powder producing cracks or other flaws which render the grid unsuitable for use.

Additionally, the use of soapstone has the disadvantage that it must be applied after each casting operation, and this adds much to the cost of the grids. On the other hand although lamp black is more durable than soapstone it has the very serious disadvantage of leaving the surface of the grid so smooth that the paste will not adhere properly to the grid.

Accordingly, it has heretofore been necessary to sand blast or otherwise roughen the grids so that the paste would properly adhere to the different parts thereof.

The objects of the present invention are to provide a coating material or compound which is inherently clean in the respect that it does not permeate the atmosphere surrounding the mold; which is more durable than the coating materials heretofore used in the sense that when applied to the faces of the mold a great many castings can be made before it is necessary to recoat the mold; which can be readily and easily applied; which gives the grid a granular surface making it possible to obtain a very effective bond between the grid and the paste which is adapted to be applied to it; and which very effectively insulates the mold from the molten metal so that good grids and other castings may be obtained without liability of the occurrence of so-called powder cracks resulting from the use of soapstone and possibly other materials.

The above and other objects are attained by my invention which may be here briefly summarized as consisting in a compound having the characteristics and composed of the ingredients which will be described in the specification and set forth in the appended claims.

Heretofore, the most refractory materials have been employed, but I depart radically from this practice by the selection of a coating material or an ingredient thereof which I believe imparts the insulating property, which under ordinary circumstances would be readily consumed or carbonized by the molten metal. I have found that certain finely ground vegetable products, when employed with a suitable binder and when applied in the right manner, answer the requirements very effectively and produce far better results than anything employed heretofore, particularly in the production of lead storage battery grids. While my experiments and extensive tests indicate that various vegetable products may be employed with varying degrees of success and efficiency, I find that a coating substance or compound consisting of finely divided cork with a binder, such as water-glass, produces the best results.

In forming this coating compound, I use a 5% to 10% solution of water-glass and mix

about equal volumes of this solution and finely divided cork, which is preferably fine enough to pass through a 100 mesh screen although the cork could still be finer.

5 This mixture is applied to a heated mold by means of a spray gun. When the spray is applied to the faces of the mold, the water in the solution is immediately vaporized with the result that the finely divided cork adheres 10 strongly to the mold faces. This result is secured by rapidly moving the spray gun over the faces of the mold, the coating operation being accomplished very quickly and without any difficulty and the coating being 15 thus evenly and thoroughly applied.

I find that contrary to what might be expected this coating is very durable and when once applied will last through far more casting operations than any prior coating material of which I am aware. Not only do the 20 finely divided cork particles adhere strongly to the faces of the mold but they resist the tendency of the molten metal to burn or carbonize them. This may or may not be 25 due to the fact that the finely divided cork particles are surrounded and possibly permeated with the binder which in itself is capable of withstanding without much deterioration the heat of the molten lead, or 30 rather lead antimony alloy.

I might state also that this coating is very cleanly and makes an exceedingly good insu-

lator, in fact it is superior both in its insulating qualities and in the prevention of adherence of the molten metal to the metal mold, 35 with the result that practically uniformly perfect grids can be produced, and the difficulties heretofore encountered because of the occurrence of cracks and other flaws is overcome. It also leaves the surface of the 40 grid in such condition that a good bond is obtained between it and the paste.

While a coating material or compound composed of powdered cork and a binder in the form of liquid glass or sodium silicate has 45 proven to have all the desired characteristics and practically none of the disadvantages of prior coating materials, I do not desire to be confined to these particular ingredients but aim in my claims to cover all modifications which do not involve a departure 50 from the spirit and scope of my invention.

Having thus described my invention, I claim:

1. A coating material for metal molds consisting of a solution containing water-glass and finely divided cork.
2. A coating material for metal molds consisting of a solution containing water glass and a finely divided vegetable substance of 60 a woody nature.

In testimony whereof, I hereunto affix my signature.

ALFRED R. WILLARD.